

# UNITED STATES PATENT OFFICE.

ARTHUR T. HINCKLEY, OF NIAGARA FALLS, NEW YORK, ASSIGNEE TO NATIONAL CARBON COMPANY, INC., A CORPORATION OF NEW YORK.

## REFRACTORY COMPOSITION AND PROCESS OF MAKING SAME.

1,346,959.

Specification of Letters Patent. Patented July 20, 1920.

No Drawing.

Application filed October 9, 1919. Serial No. 328,605.

To all whom it may concern:

Be it known that I, ARTHUR T. HINCKLEY, a citizen of the United States, residing at Niagara Falls, in the county of Niagara and State of New York, have invented certain new and useful Improvements in Refractory Compositions and Processes of Making Same, of which the following is a specification.

This invention relates to refractory bricks, blocks or other shaped articles comprising a frame-work or skeleton of fully shrunk carbon particles, and a bond of the ceramic or silicate type. My invention comprises also the carbon-containing mixture adapted for the manufacture of such shaped articles, as well as for furnace linings, hearths and the like. The invention also comprises the process by which such articles, linings or the like are prepared.

Carbon-silicate mixtures have been used or proposed for use in the manufacture of refractories, but as heretofore compounded they have not proven to possess the properties requisite where extremely high temperatures are employed. I have discovered that by the proper proportioning of the components of the mixture, the carbon component being preliminarily shrunk and graded in the proper way, as described below, it is possible to prepare from these materials a composition possessing in a very high degree those mechanical and heat-resisting qualities which are requisite for a high grade refractory.

My invention will now be described by reference to a preferred embodiment thereof, it being fully understood that the invention is not restricted to the employment of any particular grade or kind of carbonaceous material, or of ceramic bond, inasmuch as the principles involved in the preparation and compounding of the mixture are believed to be broadly novel.

I prefer to proceed as follows: I take hard coal, preferably a coal having a high density and as free as possible from laminated structure, and crush and calcine the same. The calcination is preferably carried out in an electric calcining furnace, the heating being continued until the particles are fully shrunk, in order that they may constitute the base or skeleton of a non-shrinking and permanent structure, as described below. I have found it satisfactory

for this purpose to conduct the calcination in such manner as to increase the real density of a coal from about 1.55 to approximately 2.00; or, otherwise expressed, I calcine the coal to the maximum temperature 60 which can be used without materially disintegrating or disrupting the particles or reducing their crushing strength.

For a standard 9" brick or other article having dimensions or thickness of wall of 65 a like order, I further crush the fully shrunk carbon and grade the particles to an average diameter of approximately .03". This grading may be done by screens, the selected particles being those which will pass 70 through apertures of a diameter of .04" and remain on a screen having .02" apertures. For larger articles or for thicker furnace linings or hearths the average size of the particles may advantageously be somewhat 75 increased, but so far as is practicable I use in every case uniformly sized particles. This is done in order that the voids between the particles may be determined with sufficient accuracy, and may be of such order 80 of magnitude, as to permit the proper proportioning of the components of the mixture. It is necessary therefore to avoid the admixture with the carbon particles of material proportions of carbon fines which 85 would partially fill the voids. An approximate and convenient rule for the size of particles best suited for an article of given dimensions is to increase the average diameter of the particle in proportion to the 90 increase in the dimensions of the article: thus for example for a furnace lining 4" in thickness or less, particles having an average diameter of .03" may be used (through .02" upon .02" aperture); for an 8" lining 95 .06" particles would be preferred (through .08" upon .04" aperture); and for a 12' lining, .12" particles would be selected (through .16" upon .08" aperture). It will be understood, however, that the selection of 100 these particular sizes is not essential to the practice of my invention, the essential point being that the selected particles should sufficiently approximate uniformity in dimension to provide voids having the desired volume ratio to the total volume of the carbon.

Fines, or particles having a diameter materially below .02", are not satisfactory for the purposes of this invention.

Having obtained the fully shrunk carbon 110

5 particles of the average diameter suitable for the particular use, I then determine the voids, which may readily be done by noting the volume of liquid required to fill the interstitial spaces of a given volume of the selected particles. For fully shrunk particles having the dimensions above mentioned, this interstitial volume will be found to be about 47% of the total volume occupied by the 10 particles, with a variation of perhaps 5%.

15 On the basis of the above data I prepare the refractory composition as follows: I take a known volume of the selected carbon particles and mix thoroughly that volume of clay or other bond of the ceramic type which is necessary for completely filling the voids between the carbon particles. To this mixture I add sufficient water to moisten the mass and convert it into a plastic body or heavy paste. After thorough pugging of the heavy paste it is ready for use. It is extruded under heavy pressure or otherwise shaped into the desired articles; or 20 tamped into place as a furnace lining as the case may be. After preliminarily drying, the resulting article is fired at a temperature of about 1000° C., the effect being to dehydrate the clay and to convert it into a strong bond.

25 The clay which I prefer to use is a high grade fire clay which does not fuse at the temperature mentioned, but undergoes partial or complete dehydration without material volume change but with the formation of a very strong bond, adequate for holding the 30 carbon particles in their proper position. This position is one in which the carbon particles are in mutual contact, as is obvious from the fact that the total volume of carbon particles used for a given article is sufficient 35 to fill completely the mold in which the article is made. The article comprises therefore a frame-work or skeleton of fully shrunk, graded carbon particles in mutual contact, in intimate admixture with a ceramic bonding material proportioned substantially to fill the interstitial spaces or voids between the particles. As stated above 40 the volume-ratios required to give the proper mixture are, approximately, 53 parts of graded carbon particles to 47 parts of finely ground clay. The corresponding weight-ratios are, approximately, 56 parts of graded carbon particles to 44 parts of fine clay.

45 50 55 The article prepared as above and fired to around 1000° C. possesses a distinct electrical conductivity, which may vary somewhat with the kind of carbon used, but is usually of the order of .04 ohm per CM<sup>3</sup>, specific

resistivity. It is mechanically strong, does not shrink or crack on exposure to very high furnace temperatures, and is refractory at temperatures which are quickly destructive to fire clay.

60 65 70 75 80 85 90 95 100 Owing to the manner in which the components of the composition are proportioned to each other, it is possible to heat the product without deformation to a temperature range much higher than that required for dehydrating the bond, and this may be done with advantage both as regards strength and refractory properties. For instance the article may be heated to a temperature at which incipient vitrification of the bond, or even complete vitrification occurs which for a good fire clay will be in the neighborhood of 1400° C. At still higher temperatures, attainable in the electric furnace, the silica component of the clay undergoes reduction with formation of amorphous silicon carbide. The product thus prepared is particularly desirable for crucibles. My invention includes the product irrespective of the temperature to which it is heated prior to use: in this connection it will of course be understood that the article fired to 1000° may under certain conditions of use undergo in place a further transformation to the state at which silicon carbide is present. This affords an indication of the extremely refractory character of the article.

I claim:

1. A refractory composition comprising fully shrunk, graded carbon particles in mutual contact, and a ceramic bonding material proportioned substantially to fill the interstitial spaces.

2. Process of making a refractory article comprising preparing a mixture containing fully shrunk, graded carbon particles in mutual contact, and a ceramic bonding material proportioned substantially to fill the interstitial spaces, forming the article from said mixture, and firing the same to a temperature sufficient to develop the strength of the ceramic bond.

3. Process of making a refractory article comprising preparing a mixture containing fully shrunk, graded carbon particles in mutual contact, and a ceramic bonding material proportioned substantially to fill the interstitial spaces, forming the article from said mixture, and firing the same to a temperature sufficient to develop the strength of the ceramic bond and to convert portions of the mixture into silicon carbide.

In testimony whereof, I affix my signature.

ARTHUR T. HINCKLEY.